

Jan. 10, 1939.

E. E. WICKERSHAM

2,143,812

TUNED CIRCUIT

Original Filed March 29, 1933



*Fig. 2.*



*Fig. 5.*



*Fig. 4.*



Inventor  
ELMER E. WICKERSHAM

Baldwin & Wright  
his Attorneys

## UNITED STATES PATENT OFFICE

2,143,812

## TUNED CIRCUIT

Elmer E. Wickersham, San Leandro, Calif.

Original application March 29, 1933, Serial No. 663,298. Divided and this application January 4, 1938, Serial No. 183,385

5 Claims. (Cl. 250—40)

This application is a division of my copending application Serial No. 663,298, filed March 29, 1933.

My first object of this invention is to provide a tuned circuit in which the cores of the various magnetic components of radio receiving and broadcasting sets consist of a finely divided metal having a relatively high electrical resistance, and good magnetic quality, so as to shorten the natural air gap length of the magnetic circuit in these various magnetic components of such sets.

Another object is to produce a practically closed magnetic circuit for coils and transformers of a non-corrosive, finely divided metal which may be poured dry into a coil housing to form a magnetic unit of small compact form which may be easily and cheaply constructed.

Another object is to produce a magnetic circuit of a finely divided, non-corrosive metal having high magnetic properties and whose contact resistance between the various metal particles is high enough to prevent or reduce to a minimum any eddy currents which may be induced therein.

25 A further object is to produce in a tuned circuit certain components of an electrical instrument adapted to receive short wave, broadcast, or long wave frequencies, the magnetic components of which, comprises one or more coils in each unit having a combined core and shield therefor, composed of a finely divided magnetic material such as "magnetite," which is commonly called "black sand," such as is found in large deposits along the Pacific coast and elsewhere.

I attain these objects by constructing the tuned circuit, as illustrated in the accompanying drawing, in which:

40 Fig. 1 shows a fragmentary circuit of a type to which my invention may be applied.

Fig. 2 is a vertical sectional elevation of a transformer having a single winding, a combined metallic core and shield therefor, of the loose dry type, and a housing for the core and the coil member.

45 Fig. 3 is a vertical sectional elevation of a transformer having a combined core and shield therefor, of the moulded type, enclosed in a housing.

50 Fig. 4 is a plan sectional view on line 4—4 of Fig. 3; and,

55 Fig. 5 is a vertical sectional elevation of a transformer including a "two circuit" coil which is embraced by a combined magnetic core and shield therefor, all enclosed in a housing.

In addition to these objects as set forth above, other objects will be apparent in the following specification:

I will state here and now that I am aware that metallic cores for coils and transformers have been used, including the so-called "iron clad" type of magnetic core; also, that iron cores have been and are used today in transformers employed as intermediate amplifiers in radio sets employing the superheterodyne principle; and that iron cores of the laminated type have been and are used in audio transformers, choke coils, and, in the magnetic components of loudspeakers, or reproducers; but, I am not aware that iron having the same characteristics and physical form as that of magnetite, which is generally termed in the gold mining districts, "black sand", or that magnetite or black sand has ever been used as a material to form the cores of electro-magnetic coils, transformers, loudspeakers, and especially those used in the art of manufacturing radio receiving and/or broadcasting equipment.

Referring to Fig. 1, 1—1'—1'' represent the radio frequency transformers of my preferred form as being positioned in an electrical circuit, they being particularly illustrated in Fig. 2 and Fig. 3. In Fig. 1, 2 is the audio transformer, while 3—3' represent the choke coils in this circuit and 4 represents the magnetic component of the loudspeaker or reproducer of the character illustrated in Fig. 6 of my said copending application Serial No. 663,928, allowed July 25, 1938.

Referring more particularly to Fig. 1, the first two tubes are high frequency amplifiers whereas the third tube is a detector and the fourth tube a low frequency amplifier. The input to the first tube comprises a resonant circuit made up of an inductance  $L_1$  and a condenser  $C_1$ . The input of the second tube includes the resonant circuit made up of coil  $L_2$  and condenser  $C_2$ , while the input of the third tube or detector includes the resonant circuit comprising coil  $L_3$  and condenser  $C_3$ . The three condensers  $C_1$ ,  $C_2$  and  $C_3$  are variable so that the respective circuits in which these condensers are located may be made to resonate at a predetermined carrier frequency. It should be noted that the detector tube is provided with a grid leak  $R_1$  and condenser  $C_4$  arrangement. In the circuit arrangement shown the carrier frequency is present up to the detector.

In order that others skilled in this art may make and use my invention, in spirit, I will describe the construction of the various magnetic components as set forth in the drawing.

Referring to Fig. 2, the coil member 5 is preferably formed by winding the desired number of turns of wire upon a nonconductive form, or tube, 6 and bringing the free ends of said wire 5 7-7' out through restricted tubes 8-8', to which other wires of an electrical circuit may be attached. At some desired point intermediate the ends of coil 5, a tap wire X is brought out from coil 5 through tube 8<sup>a</sup>, which may be connected 10 to a source of electrical energy, not shown. The coil is preferably supported inside of housing 9 by tubes 8-8' and 8<sup>a</sup>. It will be seen that the housing for the coil is provided with a cover 10 which is normally held in position on housing 9 15 by screws 11-11'.

In carrying out the spirit of my invention, I will assume that the coil 5 has been formed and properly insulated as at Y, by a covering of cloth, paper, or wax, and suspended in housing 9 and 20 that the cover 10 has been removed therefrom. The next step, I prefer to pour a quantity of magnetite or black sand, into housing 9, sufficient to completely submerge the coil 5 and to practically fill said housing to the top thereof, to 25 form a combined core and shield, and thus also form a "closed" magnetic circuit. The cover 10 may now be replaced on housing 9 and secured by screws 11-11' or by other means. The magnetic coil or transformer unit is now completed 30 and ready for use.

Fig. 3 shows a coil or transformer 12 having its combined core and shield formed in two parts, upper and lower, as shown at 13-13' that are composed of magnetite or black sand, which 35 has previously been wetted or moistened with a quick drying binding material such as shellac and subsequently baked to dryness in a metal mould, not shown, so that the moisture in the "binder" may be evaporated and the cores become 40 dry, hard, and self-supporting.

Each section of said core 13-13' has an annular channel 14-14' formed in the inner faces thereof, and having a central post 15 extending from the depth of said annular channel to a point 45 in the plane of said faces 16 of cores 13-13' which are adapted to support the coil 12 and its form 17 as is clearly shown in Fig. 3.

Fig. 4 shows the coil in said annular channel and also the manner in which the combined core 50 and shield of magnetite or black sand, completely engulfs and encloses the coil 12 and its form 17; it being a view taken on line 4-4 of Fig. 3.

Fig. 5 shows and illustrates a transformer of 55 the so-called audio type, the current carrying components of which are preferably formed in the two parts termed primary and secondary coils, as at 18 and 19, respectively. The combined core and shield 20 forming practically a closed 60 magnetic circuit may be formed according to the method described in the forming of the corresponding component illustrated in Fig. 2, the coils 18-19 are preferably wound on a form of insulating material 21 and then covered and 65 sealed by a flexible tubular insulating form such as shown at 22 to effectively prevent the various metallic particles which form the core and shield from making physical contact with the windings of the coils 18-19. The insulation 22 may be 70 of any suitable material such as paper.

Referring again to Fig. 5, it will be readily understood that the coil and core housing 23 is adapted to receive and enclose both the coil and core components of the transformer and 75 that a cover 24 is readily detachable so that

the said components may be readily installed and mounted therein.

One of the effects of the presence of magnetite in the field of a coil through which current is flowing, is: that for the same number of turns 5 in a coil, its inductance is increased, and consequently a coil having a closed magnetic circuit of magnetite will require a lesser number of turns of wire and proportionately reduce the ohmic resistance, which, for coils and transformers such 10 as are used in radio apparatus, is advantageous.

One advantage gained by the use of these cores for transformers when constructed of magnetite, as described, is the ease with which two or more coils may be inductively matched. The 15 magnetite, as used, is finely divided, and so pure that oxidation does not occur, and that due to the thousands of particles of the magnetite or black sand, included in a sufficient quantity of this material to make or construct a core, as 20 described, it is apparent now that by the addition of a few grains of magnetite to the core of a coil or transformer the inductance thereof will be increased, and conversely when a few grains are deleted from the core mass the in- 25 ductance of said coil will be decreased.

Thus, in order that two or more coils of the character described be made to have the same inductance, it is only necessary to either add to, or take away a sufficient quantity of magnetite or black sand from the core or one or more of said coils, to equalize their inductances. I have found by experimentation that coils having cores constructed in accordance with the spirit of my invention are very selective with 35 respect to the short wave band of radio frequencies, and I also have found that when a radio broadcast receiver having the usual multiplicity of tuned circuits and employing these coils as tuning inductances, that the selectivity 40 is adequate and the receiver is capable of operation in congested districts.

In addition to these above advantages, the tonal quality of reproduction is greatly improved, which is due in part, to the fact that all eddy 45 currents are immediately dissipated and localized by the high contact resistance between the magnetite particles forming the cores and incidental to the minute physical dimensions of the particles of magnetite used in said cores the 50 effective length of the air gap in the magnetic path is shortened and also that these cores are not easily magnetically saturated, consequently, there is no distortional effects heard 55 in the reproducer.

Inasmuch as the particular wiring scheme I have shown in Fig. 1 to illustrate the application of these various components which I have heretofore described form no part of this invention and also that the principles governing the 60 workings of the coils, transformers, and loudspeakers, or reproducers, are well understood by those skilled in this art, therefore, I deem it unnecessary to make further explanations in this regard.

I have constructed and used coils and cores in tuned circuits as described herein and am not familiar with all the phenomena which takes place therein, but I do know the results obtained by their use are indeed gratifying and I realize 70 that these cores and shields may be made in many other physical forms employing the use of magnetite, or what is known as black sand, without departing from the spirit of this invention; and, accordingly, I wish the meaning 75

and intent of the following claims to be limited only by the state of the art to which they pertain.

I claim:

- 5 1. A circuit resonant to a high carrier frequency and including an inductance coil provided with a core composed of comminuted native magnetite, retaining its native magnetic properties.
- 10 2. A circuit resonant to a high carrier frequency including an inductance coil and a condenser in circuit therewith, said inductance coil being provided with a core composed of comminuted native magnetite retaining its native magnetic properties.
- 15 3. A circuit resonant to a high carrier frequency including an inductance coil provided with a core composed of comminuted native magnetite retaining its native magnetic prop-

erties, and a condenser shunted across said inductance coil.

4. A circuit resonant to a high carrier frequency and comprising an inductance coil and an element variable to tune said circuit over 5 a band of frequencies, said coil having a core composed of comminute native magnetite mixed with a binder for maintaining the magnetite in a predetermined core shape.

5. A circuit resonant to a high carrier frequency comprising an inductance coil and a variable condenser for tuning said circuit over a band of frequencies, said coil having a core composed of comminuted native magnetite mixed with a binder for maintaining the magnetite in 15 a predetermined core shape.

ELMER E. WICKERSHAM.